

## UNITED STATES PATENT OFFICE

2,274,673

## LUBRICATING COMPOSITION

Clarence E. Earle, Washington, D. C.

No Drawing. Application April 5, 1940,  
Serial No. 328,095

10 Claims. (Cl. 252—42)

(Granted under the act of March 3, 1883, as  
amended April 30, 1928; 370 O. G. 757)

This invention relates to lubricants and process of preparing them and refers more particularly to stable grease compositions comprising an oil, a lithium soap and, if desired, stabilizing chemical compounds such as the polymerized esters of the acrylic series.

My invention provides an improved lubricating compound that is chemically and physically stable when subjected to either heat or pressure or both simultaneously.

Heretofore, lubricating greases have been manufactured and produced by compounding mineral oil and metallic salts such as sodium stearate, potassium stearate, or the oleates or other higher fatty acid salts of these two metals or alkaline earth salts of these acids such as those of calcium, barium, strontium, etc. It is significant to point out here that neither the literature nor the books on the art mention the use of lithium salts of the higher fatty acids, such as stearates, oleates, palmitates, etc., for producing greases.

I have found that the use of lithium soap or salts of soap forming higher fatty acids in the production of lubricating greases gives the greases entirely different properties from those obtained by the use of the other alkali metal salts. The greases produced by my method are water resistant, whereas the other alkali salts do not give such a property. My lithium soap greases withstand temperature greatly in excess of those containing other alkali metal salts. The properties of these improved lubricating greases are not only widely different from the other alkali metal soap types but also they are much more stable to temperature and pressure, both chemically and physically.

I have found that the addition of polymerized esters of the acrylic series materially improves the thixotropic properties of my lubricating compounds. Also I have found that the polymers of vinyl esters with long chains enhance the thixotropic properties of these improved lubricating compounds.

Various compositions of mineral oil or vegetable oil, lithium soaps and a stabilizing agent such as polymerized esters of the acrylic series can be used in production of a lubricating grease. As an example, a mixture having the following formulation limits may be employed, the percentages depending upon the type of service for which it is intended:

Percent by  
weight

Mineral oil..... 90-54  
Lithium soap or salt..... 10-40  
Polymerized esters of methacrylic acid..... 0-6

A preferred process of preparing the lubricating grease is as follows, for example: 85 parts

of a mineral oil is heated up to 130° C. to 250° C. at which temperature 14 parts of lithium stearate is added and the temperature maintained for twenty to thirty minutes. After the soap becomes thoroughly mixed with the oil, the temperature is allowed to slowly recede. At about 165° C. while the solution is still fluid one part of cetyl methacrylate is added and thoroughly stirred into the solution. The solution is allowed to cool and jell after which it is ready for use.

My invention includes the employment of polymerized esters of acrylic and methacrylic acids.

I have also found that the addition of small amounts of lithium soaps to lubricating oils improves their lubricating properties, thus lowering the power consumption and leakage from bearing interfaces.

The grease made in accordance with my invention is extremely stable both chemically and physically when subjected to either high temperature or extremely low temperature. A grease of suitable composition made in accordance with my invention will have a melting point in excess of 350° F. and still be sufficiently plastic at minus 50° F. to furnish adequate lubrication to aircraft bearings at high altitude.

The invention herein described and claimed may be used and/or manufactured by or for the Government of the United States of America for governmental purposes without the payment of any royalties thereon or therefor.

I claim:

1. A lubricating composition comprising a mineral oil, and a lithium soap of a higher fatty acid in quantity sufficient substantially to thicken said oil.

2. A lubricating composition comprising a vegetable oil and a lithium soap of a higher fatty acid in quantity sufficient substantially to thicken said oil.

3. A lubricating composition comprising a mineral oil, a lithium soap of a higher fatty acid in quantity sufficient substantially to thicken said oil and a polymerized ester of acrylic acid.

4. A lubricating composition comprising a vegetable oil, a lithium soap of a higher fatty acid in quantity sufficient substantially to thicken and a polymerized ester of acrylic acid.

5. A lubricating composition comprising oleaginous material selected from the group consisting of mineral oils and vegetable oils, a lithium soap of a higher fatty acid in quantity sufficient substantially to thicken and a polymerized ester of methacrylic acid.

6. A lubricating composition comprising oleaginous material selected from the group consisting of mineral oils and vegetable oils, a lithium soap in quantity substantially to thicken, and a polymerized vinyl ester having a hydrocar-

bon radical having an excess of 6 carbon atoms.

7. A lubricating composition comprising oleaginous material selected from the group consisting of mineral oils and vegetable oils, a lithium soap in quantity substantially to thicken, and a polymerized ester of acrylic acid.

8. As a new composition of matter, a lubricating grease comprising 54 to 90 parts of an oleaginous material selected from the group consisting of mineral and vegetable oils, 10 to 40 parts of a lithium soap of a higher fatty acid, and not more than 6 parts of a polymerized long-chained ester of methacrylic acid.

9. As a new composition of matter, a lubricating grease comprising 54 to 90 parts of a mineral oil, 10 to 40 parts of a lithium soap of a higher fatty acid, and not more than 6 parts of a polymerized long-chained ester of methacrylic acid.

10. As a new composition of matter, a lubricating grease comprising a lithium soap and a lubricating oil from the class consisting of mineral and vegetable oils, said lithium soap being present in quantities sufficient substantially to thicken the oil.

CLARENCE E. EARLE.